

## UNITED STATES PATENT OFFICE.

WILLIAM A. FARISH, OF BUFFALO, NEW YORK, ASSIGNOR TO BUFFALO REFRACRYOR CORPORATION, OF BUFFALO, NEW YORK, A CORPORATION OF DELAWARE.

## METHOD OF MAKING REFRACRYOR PRODUCTS AND ARTICLES PRODUCED THEREBY.

No Drawing.

Application filed August 31, 1922, Serial No. 585,522.

The general object of this invention is to provide a simple and effective method of forming refractory products in such a way as to make them durable and prevent cracking, disintegration, corrosion, and oxidization.

Moreover, my object has been to provide a method which can be asily and cheaply performed, and one which will make it unnecessary to raise the temperature to which the 10 composition is subjected above that of recrystallization.

By using the method of my invention, I am able to create a product, which resists chemical action and which greatly increases 15 the life of articles made in accordance with my invention.

By means of my method any heat resisting articles may be made such as crucibles, fire-bricks, retorts, furnace cores, tubes, furnace 20 linings, combustion boats, heat resisting cements, and any other form of product, which is subjected to very high temperatures.

In describing my method, it is to be understood that the exact proportions of elements entering into the composition and the exact sequence of steps performed in following the invention are only preferably stated and some modifications may be used which will attain the desired objects without departing from the spirit of the invention as 30 herein disclosed.

In general, I first make a dry mixture of graphite, and a suitable electric furnace refractory product with or without a suitable 35 solid fluxing agent. This compound is thoroughly mixed. Then a suitable carbonizing binder is added and the mixture is thoroughly impregnated with it until all of the ingredients of the compound have been intimately mixed together. Then I mold this 40 compound in any suitable way and under any suitable pressure. The compound is then placed in a carbonizing kiln, and subjected to a temperature which will thoroughly carbonize it. While the compound, 45 so carbonized, is still warm, it is dipped into a liquid fluxing agent. After being dipped it is subjected to a high temperature in a suitable annealing furnace.

50 Preferably in the dry mixture, I employ about 17% of graphite; about 12% of silica, and about 71% of silicon-carbide. While these are the preferable proportions of the elements of this dry mixture, still it is to be

understood that for some purposes a satisfactory product may be obtained by employing a maximum of 55% and a minimum of 10% of graphite in such mixture; a maximum of 25% and a minimum of 5% of the fluxing agent; and a maximum of 75% and 55 a minimum of 20% silicon-carbide.

For the solid fluxing agent feldspar or some other suitable agent may be employed. In place of the silicon-carbide any electric furnace refractory product such as fused 60 magnesite, fused aluminum oxide, or fused silica may be used with satisfactory results. In such cases the proportions as to maximums and minimums of these substitute elements will be substantially as hereinbefore 65 stated.

For the carbonizing binder, molasses, pitch or tar may be employed. If molasses is employed, I preferably use about 15%, but a maximum of 40% and a minimum of 10% of 70 this binder may be advantageously used. If pitch is employed, the preferable amount is about 20% but a maximum of 50% or a minimum of 8% may be advantageously used. If tar is used, the preferable amount 75 should be about 15% but a maximum of 40% and a minimum of 10% can be advantageously used. It is to be understood that molasses, tar and pitch are only examples of suitable carbonizing binders, and that other 80 carbonizing binders than those named can be advantageously used within the limits of maximums and minimums above set forth.

After removing the product from the carbonizing kiln, it is dipped, preferably while 85 it is warm, into a liquid fluxing agent, such as sodium borate or sodium silicate.

After being dipped the product is placed in an annealing furnace, and is preferably subjected to a heat of substantially 1200° F. 90

In carrying out my invention as hereinbefore described, I have found that the products formed and treated according to my disclosure will withstand extremely high temperatures and rough handling without material damage.

Having thus described my invention what I claim is:

1. A method of making refractory products comprising forming an intimate dry 105 mixture of graphite, and an electric furnace refractory product, then intimately impregnating such dry mixture with a carbonizing

binder, then forming the product, then carbonizing the product, and then dipping the product into a liquid fluxing agent.

2. A method of making refractory products comprising forming an intimate dry mixture of graphite, a solid fluxing agent, and an electric furnace refractory product, then intimately impregnating such dry mixture with a carbonizing binder, then forming the product, then carbonizing the products, and then dipping the product into a liquid fluxing agent. 70

3. A method of making refractory products comprising forming an intimate dry mixture of graphite, and an electric furnace refractory product, then intimately impregnating such dry mixture with a carbonizing binder, then forming the product, then carbonizing the product, then dipping the product into a liquid fluxing agent, and then subjecting the product to a suitable heat in an annealing furnace. 80

4. A method of making refractory products comprising the formation of an intimate dry mixture of substantially 17% of graphite, substantially 12% of a suitable solid fluxing agent; and substantially 71% of an electric furnace refractory product, then intimately mixing with the dry mixture a quantity of carbonizing binder equal to substantially 15% of the dry mixture, then forming the product, then carbonizing such product, and then dipping the product into a liquid fluxing agent. 95

5. A method of making refractory products comprising the formation of an intimate dry mixture of substantially 17% of graphite, substantially 12% of a suitable solid fluxing agent, and substantially 71% of an electric furnace refractory product, then intimately mixing with the dry mixture a quantity of carbonizing binder equal to substantially 15% of the dry mixture then forming the product, then carbonizing such product, and then dipping the product, while still warm, into a saturated solution of a fluxing salt. 100

6. A method of making refractory products comprising the formation of an intimate dry mixture of substantially 17% of graphite, substantially 12% of a suitable solid fluxing agent, and substantially 71% of an electric furnace refractory product, then intimately mixing with the dry mixture a quantity of carbonizing binder equal to substantially 15% of the dry mixture, then forming the product, then carbonizing such product, then dipping the product into a liquid fluxing agent, and then subjecting the product to heat in an annealing furnace. 115

7. A method of making refractory products comprising the formation of an intimate dry mixture of substantially 17% of graphite, substantially 12% of a suitable solid fluxing agent, and substantially 71% 125

of an electric furnace refractory product, then intimately mixing with the dry mixture a quantity of carbonizing binder equal to substantially 15% of the dry mixture, then forming the product, then carbonizing such product, then dipping the product into a liquid fluxing agent, and then subjecting such product to a heat of substantially 1200° F. in a suitable annealing furnace. 130

8. A method of making refractory products comprising the formation of an intimate dry mixture of not more than 55% and not less than 10% of graphite, and not more than 75% and not less than 20% of an electric furnace refractory product, then intimately mixing with the dry mixture a quantity of carbonizing binder equal to not more than 50% and not less than 8% of the dry mixture, then forming the product, then carbonizing such product, and then dipping such product into a suitable liquid fluxing agent. 140

9. A method of making refractory products comprising the formation of an intimate dry mixture of not more than 55% and not less than 10% of graphite, not more than 25% and not less than 5% of a suitable solid fluxing agent, and not more than 75% and not less than 20% of an electric furnace refractory product, then intimately mixing with the dry mixture a quantity of carbonizing binder equal to not more than 50% and not less than 8% of the dry mixture, then forming the product, then carbonizing such product, and then dipping such product into a suitable liquid fluxing agent. 150

10. A method of making refractory products comprising the formation of an intimate dry mixture of not more than 55% and not less than 10% of graphite, not more than 25% and not less than 5% of a suitable solid fluxing agent, and not more than 75% and not less than 20% of an electric furnace refractory product, then intimately mixing with the dry mixture a quantity of carbonizing binder equal to not more than 50% and not less than 8% of the dry mixture, then carbonizing such product, then forming the product, then dipping such product into a suitable liquid agent, and then subjecting such product to heat in a suitable annealing furnace. 160

11. A method of making refractory products comprising the formation of an intimate dry mixture of not more than 55% and not less than 10% of graphite, not more than 25% and not less than 5% of a suitable solid fluxing agent, and not more than 75% and not less than 20% of an electric furnace refractory product, then intimately mixing with the dry mixture a quantity of carbonizing binder equal to not more than 50% and not less than 8% of the dry mixture, then forming the product, then carbonizing such product, then dipping such product, while

still warm, into a suitable liquid fluxing salt, and then subjecting the product to a temperature of substantially 1200° F. in a suitable annealing furnace.

- 5 12. A dense hard refractory graphitic article of manufacture having a body bond and a continuous glaze of non-ceramic material and of the same coefficient of expansion and other physical characteristics.
- 10 13. In the art of making graphitic refractory articles containing a refractory the im-

provement which consists in diffusing silicon throughout the pores of the article by incorporation and heating, converting the diffused silicon into silicate by treating the 15 article with an alkali, and exuding the silicate to the surface of the article by the application of heat.

In testimony whereof, I have hereunto signed my name.

WILLIAM A. FARISH.